



US005096466A

**United States Patent** [19]

Satake et al.

[11] **Patent Number:** **5,096,466**[45] **Date of Patent:** **Mar. 17, 1992**[54] **ABRASIVE ROLL AND METHOD OF PRODUCING THE SAME**[75] Inventors: **Toshihiko Satake, Higashihiroshima; Satoru Satake, Tokyo; Takamasa Mesaki, Hiroshima, all of Japan**[73] Assignee: **Satake Engineering Co., Ltd., Tokyo, Japan**[21] Appl. No.: **588,104**[22] Filed: **Sep. 25, 1990****Related U.S. Application Data**

[63] Continuation of Ser. No. 380,170, Jul. 14, 1989, abandoned.

**Foreign Application Priority Data**

Jul. 19, 1988 [JP] Japan ..... 63-181298

[51] Int. Cl.<sup>5</sup> ..... B24D 3/00

[52] U.S. Cl. ..... 51/296; 51/307; 51/308; 51/309

[58] Field of Search ..... 51/296, 307, 308, 309

[56]

**References Cited****U.S. PATENT DOCUMENTS**

|           |         |                      |        |
|-----------|---------|----------------------|--------|
| 3,416,905 | 12/1968 | Waugh .....          | 51/296 |
| 4,086,067 | 4/1975  | Busch et al. .....   | 51/309 |
| 4,494,964 | 1/1985  | Ohlsson et al. ..... | 51/296 |
| 4,997,460 | 3/1991  | Satake et al. .....  | 51/296 |

*Primary Examiner*—William R. Dixon, Jr.  
*Assistant Examiner*—Willie J. Thompson  
*Attorney, Agent, or Firm*—Darby & Darby

[57] **ABSTRACT**

A method of producing an abrasive roll comprises the steps of forming a mixture of substances such as abrasive grains, a bond, a temporary caking agent and a pore forming agent, molding the mixture into a body having a predetermined shape, and drying and then burning the body. The pore forming agent is constituted from a rice hull powder sieved to have a predetermined particle size, thereby enabling to produce an abrasive roll of high porosity which has pores having substantially ball-like shape and substantially uniform size and includes a bond having portions of high SiO<sub>2</sub> concentration each adjacent to and surrounding one of the pores.

**11 Claims, No Drawings**

## ABRASIVE ROLL AND METHOD OF PRODUCING THE SAME

This is a continuation under 37 CFR 1.60 of U.S. patent application No. 380,170 of Toshihiko Satake, Saturo Satake and Takamasa Mesake entitled "Abrasive Roll and Method of Producing Same", filed on July 14, 1989, now abandon.

### BACKGROUND OF THE INVENTION

#### 1. Field of the Invention

The present invention relates to an abrasive roll and a method of producing the same.

#### 2. Description of the Prior Art

It has hitherto been known that a method of producing an abrasive roll for use with rice polishing machines, for example, ordinarily comprises the step of forming a mixture of substances such as abrasive grains, a bond and a temporary caking agent, and that the formation of the mixture is effected, taking amounts or proportions of these respective substances into consideration. Also it has been known that a powder or a dust of substances such as polystyrene, foamed styrol, wood, cork and walnut is sometimes added into the mixture as a pore forming agent.

The abrasive roll produced without using the pore forming agent has a low porosity and suffers from an inferior polishing efficiency. When the grain percentage of an abrasive roll is increased with a view to attaining an improved polishing efficiency, the grade of the abrasive roll lowers. The abrasive roll having a low grade is impossible to be used for the rice polishing since partial wear thereof would occur during the polishing operation. Further, in the case where the powder or the dust of the abovementioned substances is used as the pore forming agent, it is difficult to enhance strength of the bond bridging and bonding the abrasive grains and hence to enhance the grade of the abrasive roll. The abrasive roll having the bond of low strength can be used for polishing rice at high efficiency only at an initial stage of the rice polishing operation. Since the strength of the bond and hence the grade are low, the bond may be broken, causing abrasive grains to be separated from the abrasive roll. This makes the surface portion of the abrasive roll rough and disadvantageously causes broken rice grains to be produced during the rice polishing.

The porosity of an abrasive roll may be increased by adjusting the molding pressure. However, the molding pressure adjustment is not effective for forming pores of uniform size and for preventing formation of pores of large size more than 500  $\mu\text{m}$ . The polishing with the use of the abrasive roll with the pores of such large size may disadvantageously cause the rice grains to be broken.

### SUMMARY OF THE INVENTION

It is therefore an object of the invention to provide an abrasive roll which may be preferably used for the rice polishing without accompanying the disadvantages of the prior art described hereinabove.

It is another object of the invention to provide a method of producing such abrasive roll.

According to an aspect of the invention, there is provided a method of producing an abrasive roll comprising: forming a mixture of abrasive grains, a bond, a temporary caking agent and a pore forming agent, said pore forming agent essentially consisting of a rice hull

powder sieved to have a predetermined particle size; molding the mixture into a body having a predetermined shape; and drying and then burning the body.

According to another aspect of the invention, there is provided an abrasive roll produced by such method.

The above and other objects, characteristic features and advantages of the invention will become more apparent from the description on an embodiment of the invention given hereinafter.

10

### DETAILED DESCRIPTION OF THE EMBODIMENT

An embodiment of the invention will be described hereunder.

15 In this embodiment, abrasive grains may be constituted from such substances as SiC (silicon carbide) and  $\text{Al}_2\text{O}_3$  (alumina), and a powder of such substances as feldspar, pottery stone and clay may be used as a bond i.e. burnable. A temporary caking agent may be constituted by starch obtained from potatoes. Further, a pore forming agent is constituted from a powder of rice hull sieved to have a predetermined particle size which is appropriately selected in consideration of a use of an abrasive roll to be produced.

20 In this embodiment, the abrasive grains, bond, pore forming agent and temporary caking agent are mixed together and agitated in a mixing machine. For example, 100 weight parts of the abrasive grains, 50 weight parts of the bond, 3 to 8 weight parts of the pore forming agent, 0.8 weight parts of the temporary caking agent and about 12 weight parts of cold and hot waters are mixed together and agitated. For example, 30- to 60-mesh powder of rice hull is used as the latter pore forming agent for producing in an abrasive roll pores of the corresponding size.

25 A mixture obtained by the abovementioned mixing and agitating process is sieved with the use of a swingable sieve to have a predetermined particle size, and then pressed as being gradually flown into a metal mold of a suitable shape placed in a molding machine. A molded body formed by the molding operation in the molding machine is then placed in a drying furnace and dried therein for about two days by a hot air in the furnace which has a temperature of about 80° to 90° C. Thereafter, the molded body is burnt or fired in a burning or firing furnace continuously for about 70 hours. In the burning furnace, the molded body is burnt at gradually increased temperatures, and near the final stage of the burning process the temperature reaches about 40 1300° C. and the molded body is burnt at the latter temperature firing the final stage for 1 to 8 hours. The molded body thus burnt is dried under the atmosphere for about one week, and then an outer periphery thereof and the other parts required are cut and ground to obtain an abrasive roll constituting a final product.

50 It is to be noted that the rice hull powder constituting the pore forming agent consists of substances such as cellulose, lignin, hemicellulose, hydrocarbon and silica. When the hull powder is burnt, gases such as  $\text{N}_2$ ,  $\text{CO}$ ,  $\text{CO}_2$ ,  $\text{H}_2$ ,  $\text{CH}_4$ ,  $\text{C}_2\text{H}_4$ , and  $\text{O}_2$  are generated. An amount of ash produced by the burning of the hull powder is about 16% by weight of the hull powder to be burnt. The produced ash contains  $\text{SiO}_2$  in an amount of about 95% by weight of the entire ash, and the balance consisting of substances such as  $\text{CaO}$ ,  $\text{MgO}$ ,  $\text{Na}_2\text{O}$ ,  $\text{Fe}_2\text{O}_3$  and  $\text{P}_2\text{O}_5$ .

55 Since the gases are generated during burning of the hull powder, an abrasive roll of high porosity may be

produced. Further, the pores formed in a structure of the abrasive roll have spherical or substantially ball-like shape and substantially uniform size or diameter. Furthermore, since  $\text{SiO}_2$  in the abovementioned amount is contained in the ash produced by the burning of the hull powder, the concentration of  $\text{SiO}_2$  at the portions of the bond each adjacent to and surrounding one of the pores, i.e., at interfaces between the pores and the bond, is enhanced. Consequently, an abrasive roll of high porosity which has a high bond strength and a high grade may be produced. Since the abrasive roll produced has a high bond strength and a high grade it is suitable to use as an abrasive roll for the rice polishing for which high strength and improved grinding properties are required. Further, according to the invention, it is possible to produce an abrasive roll for the precision grinding by using as the pore forming agent the hull powder sieved to have a particle size appropriate for this purpose.

As will be apparent from the foregoing description, according to the invention, a rice hull powder sieved to have a predetermined particle size is used as a pore forming agent. This enhances the porosity of the abrasive roll produced, and hence improves polishing efficiency of the abrasive roll by preventing the pores from being clogged with dusts produced by the polishing operation. Further, since the abrasive roll according to the invention has high  $\text{SiO}_2$  concentration at the interfaces between the bond and the pores, the strength of the bond and the grade are increased and hence separation of the abrasive grains from the abrasive roll is suppressed. Furthermore, the pores have substantially ball-like shape and uniform size. Consequently, the abrasive roll fit for various uses requiring improved grinding properties may be obtained. For example, the abrasive

roll which may be preferably used for the rice polishing without producing broken rice grains is obtainable.

What is claimed is:

1. A precursor for forming an abrasive roll, comprising:  
an abrasive grain;  
a bonding material;  
a temporary caking agent; and  
a pore forming agent sieved to a particular particle size, the pore forming agent producing substantially uniformly sized and shaped pores when the roll is dried and burned.
2. The precursor for forming an abrasive roll of claim 1, wherein the abrasive grain includes silicon carbide.
3. The precursor for forming an abrasive roll of claim 1, wherein the pore forming agent produces gases when burned, the gases forming spherical pores in the abrasive roll.
4. The precursor for forming an abrasive roll of claim 20, wherein the pore forming agent is rice hull powder.
5. The precursor for forming an abrasive roll of claim 1, wherein the bonding material and temporary caking agent are burned off when the roll is burned.
6. The precursor for forming an abrasive roll of claim 25, wherein the temporary caking agent is potato starch.
7. The abrasive roll of claim 1, wherein the mixture comprises 3-8 parts of the pore forming agent per 100 parts of abrasive grains by weight.
8. The abrasive roll of claim 1, wherein the abrasive 30 grain comprises silicon carbide.
9. The abrasive roll of claim 1, wherein the abrasive grain comprises alumina.
10. The abrasive roll of claim 1, wherein the temporary caking agent is potato starch.
11. The abrasive roll of claim 7, wherein the mixture further comprises, by weight, 50 parts bonding material and 0.8 parts temporary caking agent.

\* \* \* \* \*

UNITED STATES PATENT AND TRADEMARK OFFICE  
CERTIFICATE OF CORRECTION

PATENT NO. : 5,096,466  
DATED : September 25, 1990  
INVENTOR(S) : Toshihiko SATAKE, ET AL.

It is certified that error appears in the above-identified patent and that said Letters Patent is hereby corrected as shown below:

On the patent cover in the "Related U.S. Application Data" (item 63), change:  
"Continuation of Ser. No. 380,170, Jul. 14, 1989, abandoned." to --Continuation of Ser. No. 380,170, Jul. 14, 1989, which issued as U.S. Patent No. 4,997,460 on Mar. 5, 1991.--

Col. 1, line 1, change "now abandoned" to  
--which issued on March 5, 1991 as  
U.S. Patent No. 4,997,460--.

Signed and Sealed this  
Twentieth Day of September, 1994

Attest:



BRUCE LEHMAN

Attesting Officer

Commissioner of Patents and Trademarks